

## [54] METHOD OF MAKING A COMPOSITE STEEL TUBING

[75] Inventor: John J. Arntz, Shelby, Ohio

[73] Assignee: Copperweld Steel Company, Shelby, Ohio

[22] Filed: Jan. 22, 1974

[21] Appl. No.: 435,526

## Related U.S. Application Data

[63] Continuation of Ser. No. 295,993, Oct. 10, 1972, abandoned, which is a continuation-in-part of Ser. No. 126,633, March 22, 1971, abandoned.

[52] U.S. Cl. .... 29/516, 29/520, 29/523, 138/151

[51] Int. Cl. .... B21d 39/00, B23p 11/00

[58] Field of Search .... 29/516, 520, 523 X; 138/140, 151 X

[56]

## References Cited

## UNITED STATES PATENTS

|           |         |                   |           |
|-----------|---------|-------------------|-----------|
| 1,441,459 | 1/1923  | Small .....       | 138/51    |
| 1,839,964 | 1/1932  | Harvey .....      | 29/516 UX |
| 2,063,325 | 12/1936 | McLeod .....      | 138/140   |
| 2,198,149 | 4/1940  | Bangert .....     | 29/516    |
| 2,219,434 | 10/1940 | White .....       | 29/516 UX |
| 3,461,523 | 8/1969  | Peehs et al. .... | 29/516 X  |

3,532,476 10/1970 Peehs et al. .... 29/516 X

## FOREIGN PATENTS OR APPLICATIONS

822,983 1/1938 France .....

858,615 1/1952 Germany .....

Primary Examiner—Charlie T. Moon

Attorney, Agent, or Firm—Buell, Blenko &amp; Ziesenhein

[57]

## ABSTRACT

The specification discloses a double wall steel tubing and a method of making it which results in the production of steel tubing having a size range and wall thickness heretofore available only in a seamless tubing and possessing a uniformity of wall thickness within heretofore unattained tolerance limits. An outer welded tube is first telescoped over an inner welded tube. The two tubing sections are then mechanically bonded together as by being drawn through a sizing die in a sink pass without a mandrel or by forcing a mandrel through the inner tubing section. The composite tubing is then drawn through a second sizing die over a mandrel to produce a heavy wall tubing, equivalent in strength characteristics to single wall tubing of the seamless type.

14 Claims, 4 Drawing Figures



PATENTED FEB 4 1975

3,863,328

SHEET 1 OF 2

Fig. 1.



Fig. 2.



Fig. 3.



INVENTOR

John J. Arntz

*Spaul, Blenko & Zelen Inc.  
his attorney*

PATENTED FEB 4 1975

3,863,328

SHEET 2 OF 2

Fig. 4.



## METHOD OF MAKING A COMPOSITE STEEL TUBING

The present application is a continuation of my prior application, Ser. No. 295,993, filed Oct. 10, 1972, now abandoned, which application in turn is a continuation-in-part of my prior application, Ser. No. 126,633, filed Mar. 22, 1971, now abandoned.

This invention relates to composite steel tubing having a degree of wall thickness not heretofore available except in steel tubing of the seamless type, and to a method of making such composite steel tubing.

Seamless tubing is produced according to present-day methods by a process involving heating a solid tube round to a forging temperature and then forcing it with a rotary motion over a piercing point to form a hollow for subsequent cold drawing. Because it is impossible to keep the piercing point always in the exact center of the tube round during the piercing operation, a wall thickness variation or eccentricity often results. Moreover, since the tube is turning as it is being formed, a spiraling eccentricity of wall thickness may be produced. This lack of uniformity of wall thickness may be greatly reduced or refined by subsequent hot and cold finishing operations but the eccentricity is never fully eliminated.

Where tolerance limits of wall thickness permit, seamless tubing may be employed, especially in the larger size ranges. However where the application requires tubing having more exacting or restrictive tolerances of wall thickness, additional processing of the seamless tubing is required, such as machining or grinding. This additional processing is, however, impractical except in relatively short sections.

An alternative process of making high-strength tubing is the cold drawing over a mandrel of electric resistance welded tubing. This process produces a tubing comparable in strength to the seamless tubing and characterized by a greater uniformity of wall thickness. However this process has its limitations in that tubing, having wall thicknesses exceeding dimensions of the order of 0.340 inch, is not presently practical by this method.

In accordance with the present invention, it is proposed to provide a method for producing tubing in larger diameter ranges and greater wall thicknesses than has heretofore been attainable by known cold-drawing processes and equal in wall thickness to tubing of the seamless type. More specifically, it is proposed to produce tubing having wall thicknesses up to twice that presently available by the cold drawing process by the employment of a "double-wall" concept in which an inner tubing and an outer tubing of the same metal such as steel, are telescoped and joined into an integral tubing. This concept has been utilized variously with tubing of different metals for the purpose of providing a relatively thin layer or protective layer within or outside a relatively thick walled tubing, where the purpose of the liner is primarily for protection against chemical action or corrosion and not for the addition of physical strength.

Many of the various processes by which such double-walled tubing of dissimilar metals are produced involve a metallurgical union or a bonding with a bonding agent of the liner to the basic tubing via a heating stage. As an example, there is described in U.S. Pat. No. 2,371,348 to M. G. Murray a process for making a composite tubing by heating telescoped sections of tub-

ing of different metals to fuse a bonding agent applied therebetween, followed by insertion of a cold bar inside the inner tubing section, while still hot, to prevent separation of the outer and inner tubing sections, as cooling progresses, due to the differing temperature coefficients of expansion of the different metals.

Similarly there is described in U.S. Pat. No. 2,219,434 to H. N. White a process for making a composite tubing having an outer tubing section of nickel silver and an inner tubing section of sterling silver, which process involves a single pass of cold drawing the telescoped tubing sections through a die and over a mandrel to effect union of the two tubing sections.

The process proposed, according to the present invention, differs from heretofore known methods of making composite tubing by reason of the fact that both outer and inner tubing sections are of the same metal, such as steel, and differences in the temperature coefficient of expansion of the telescoped tubing sections do not present a problem to be dealt with. Moreover, absence of any requirement for a bonding agent between the tubing sections, simplifies the process and avoids problems arising out of heating the assembled tubing sections.

More specifically, the proposed process involves the provision of two tubing sections of such different diameters as to enable one tubing section to be telescoped within the other, the mechanical bonding of the two tubing sections by altering the diameter of one of the tubing sections relative of that of the other tubing section, and the cold drawing of the united tubing sections through a die and over a mandrel to size the final product.

Alteration of the diameter of one of the tubing sections is effected either by cold drawing the telescoped tubing sections without lubrication or the use of a bonding agent therebetween, through a die and without a mandrel to compress the outer tubing section on the inner tubing section into close contact or by cold drawing a mandrel or plug through the inner tubing section to expand it into contact with the outer tubing section.

The proposed process thus provides a practical method for making tubing having heavy wall thicknesses conforming to heretofore unattained tolerances without requiring any special cold drawing equipment other than has heretofore been employed for tubing of lesser thicknesses.

The method for producing a composite tubing according to the present invention will be described more fully hereinafter in connection with the accompanying drawings, wherein:

FIG. 1 is a longitudinal sectional view, showing outer and inner tubing sections telescoped and hammered at one end preparatory to sink drawing;

FIG. 2 is a longitudinal sectional view, showing the composite tubing after sink drawing through a die without a mandrel;

FIG. 3 is a longitudinal sectional view, showing the composite tubing after cold drawing through a sizing die and over a mandrel; and

FIG. 4 is a longitudinal sectional view showing an alternative step to that of FIG. 2.

As will be apparent by reference to FIG. 1, the initial step in pursuing the process here disclosed is to select two sections of normalized welded steel tubing respectively having appropriate length such as 20 to 30 feet, outside diameter, inside diameter and wall thickness to

produce the ultimate product desired. As a matter of convenience and brevity the term "outside diameter" will be referred to hereafter as "O.D.", the term "inside diameter" will be referred to as "I.D." and the term "wall thickness" will be referred to as "W.T.". Let it be assumed, for example, that two tubing sections 10 and 11 have been selected with the following dimensions:

| Tubing | O.D. | I.D.  | W.T.  |
|--------|------|-------|-------|
| 10     | 7.5" | 6.75" | .375" |
| 11     | 6.5" | 5.75" | .375" |

It will be noted that there is a total clearance of 0.25 inch between the I.D. of tubing 10 and the O.D. of tubing 11, thereby enabling the two tubings to be readily telescoped completely as shown in FIG. 1, which is the first step in the process. The tubes are now hammered or flattened at one end with the inner tubing 11 extending slightly outside of the outer tubing 10 and flared so as to firmly lock the two tubes 10 together. Also, the "open end" of the inner tubing 11 is extended an amount, such as 12 to 18 inches, beyond the outer tubing 10 to compensate for the fact that the outer tube will elongate or "grow" in length to a greater extent than the inner tubing during the initial cold drawing stage or "sink pass," now to be described.

Referring to FIG. 2, the sink pass consists of cold drawing the hammered or flattened ends of the telescoped sections of tubing through a die 12, which in the case of the original or starting dimensions for example, reduces the outer tubing to a 7 inch O.D. Assuming that the wall thickness of the outer tubing remains unchanged at 0.375 the resultant I.D. for the outer tubing would be 6.25 inches. Since no mandrel is employed inside the inner tubing for this stage of the process, the operation is termed "sink" drawing. It will be understood that in consequence of this operation the outer tubing is reduced circumferentially and diametrically and coincidentally compressed tightly over and around the inner tubing. However, with the assumed tubing dimensions the O.D. of the inner tubing is larger than the assumed resultant I.D. of the outer tubing. Accordingly, to accommodate the situation, the outer tubing is elongated and the inner tubing becomes smaller in diameter. This adjustment is shown in FIG. 2, where the "open" end of the outer tubing 10 is shown as shifted to the right relative to the open end of the inner tubing. At this particular stage of the process, it might be said that the tubing sections, theoretically at least, form a composite tube with a 7 inch O.D. and 0.75 inch W.T.

In order to avoid impairment of the mechanical bond between the I.D. surface of the outer tubing and the O.D. surface of the inner tubing, no lubricant is applied to the tubing sections prior to the sink pass of FIG. 2, except that the O.D. surface of the outer tubing is lubricated.

The next step in the process involves cold drawing the composite tubing simultaneously through a die 13 and over a mandrel 14, as shown in FIG. 3. Preceding this cold drawing operation, the composite tubing is dipped into a lubricant, without annealing the tubing however. Following the heretofore assumed dimensional relations of the tubing sections 10 and 11, die 13 may be such as to produce a 6.5 inch O.D. for the outer tubing 10 and the mandrel 14 may be such as to pro-

duce a 0.668 W.T. thus resulting in an I.D. of 5.125 inches for the inner tubing section 11, which correspondingly elongates relative to the outer tubing section.

5 A variation of the process may be followed which involves substituting the step shown in FIG. 4 for the step shown in FIG. 2.

As will be apparent from the drawing, the step of FIG. 4 involves expansion of the inner tubing section 11 into contact with the outer tubing section 10 to effect a mechanical bond therebetween. This is accomplished in the manner illustrated by FIG. 4, that is, by pulling an appropriately sized mandrel 15 in the right-hand direction through the inner tubing section 11 to 15 expand it circumferentially into contact with the inner diameter of the wall of the outer section 10. On the basis of the original tubing dimensions, the outer diameter of the inner tubing section will be expanded 0.25 inch to match the I.D. of 6.75 inches of the outer tubing section. 20 Assuming no expansion of the outer tubing section 10, the resultant O.D. for the composite tubing would be 7.5 inches. If diametrical expansion of the inner tubing section occurs beyond that necessary to effect a mechanical bond, then some lengthwise expansion 25 of the inner tubing section will occur. It will be understood, therefore, that if it is desired to arrive at the same ultimate O.D. for the composite pipe while employing the step of FIG. 4 as for the step of FIG. 2, a correspondingly reduced O.D. of the outer tubing section 30 must be employed at the start.

A further variation of the above described process may be followed, where further improvement in the mechanical bond between the tubing sections is desired. In this variation, the I.D. surface of the outer tubing section is "picked," that is, scored prior to the initial telescoping of the tubing sections. This scoring operation may be accomplished by pulling a tool through the inside diameter of the outer tubing section. An example of a tool suitable for this purpose is described and claimed in U.S. Pat. No. 3,504,513, assigned to the assignee of this application. In consequence of the scoring of the inside diameter surface of the outer tubing section, the O.D. surface of the inner tubing section is interlockingly impressed into the scored indentations of the I.D. surface of the outer tubing section, thus providing a more effective mechanical bond between the two tubing sections.

In the alternative, the O.D. surface of the inner tubing section may be scored prior to the original telescoping of the tubing sections. This can be accomplished incidentally to the process of making the tubing section itself. The effect is the same as before, namely an improvement in the mechanical bond between the tubing sections of the composite tubing made in accordance with the hereinbefore described process.

Tests conducted on samples of the composite tubing produced according to the herein described process have established that in both tensile and burst strength values, the composite tubing is the equivalent in performance to seamless tubing of similar dimensions.

It is to be understood that no limitations are intended with respect to the sizes of tubing which may be made by the foregoing process. However, the particular utility and advantage of the process lies in producing composite tubing of heavy wall thickness to heretofore unattained tolerance limits.

I claim:

1. The method of making a composite steel tubing comprising the steps of:

- a. providing two sections of welded steel tubing of substantially equivalent wall thickness, one of which sections has an outer diameter less than the inner diameter of the other;
- b. telescoping said tubing sections and locking them together at one end;
- c. cold drawing said telescoped tubing sections through a die without a mandrel to compress the outer tubing section onto the inner tubing section thereby to produce a mechanical bond therebetween; and
- d. cold drawing the united tubing sections through a sizing die and over a mandrel.

2. The method of making a composite steel tubing according to claim 1, wherein the sum of the wall thicknesses of the two tubing sections provided exceeds 0.340 inch.

3. The method of making a composite steel tubing according to claim 1, wherein one of the tubing sections provided has its mating surface scored prior to telescoping the tubing sections.

4. The method of making a composite steel tubing according to claim 1, wherein the outer diameter surface of the inner tubing section is scored prior to telescoping the tubing sections.

5. The method of making a composite steel tubing according to claim 1, wherein the inner diameter surface of the outer tubing section is scored prior to telescoping the tubing sections.

6. The method of making a composite steel tubing comprising the steps of:

- a. providing two sections of welded steel tubing of substantially equivalent wall thickness, one of which sections has an outer diameter less than the inner diameter of the other;
- b. telescoping said tubing sections and holding them together at one end;
- c. changing the diameter of one of said tubing sections so as to produce a mechanical bond therebetween; and
- d. cold drawing the united tubing sections through a sizing die and over a mandrel.

7. The method of making a composite steel tubing ac-

cording to claim 6, wherein the change in the diameter of one of said tubing sections is accomplished by cold drawing the telescoped tubing sections through a die without a mandrel to compress the outer tubing section onto the inner tubing section.

8. The method of making a composite steel tubing according to claim 6, wherein the change in the diameter of one of said tubing sections is accomplished by expanding the inner one of said tubing sections.

9. The method of making a composite steel tubing according to claim 6, wherein the expansion of the inner one of said tubing sections is accomplished by forcing a mandrel therethrough.

10. The method of making a composite steel tubing according to claim 6, wherein the sum of the wall thicknesses of the two tubing sections provided exceeds 0.340 inch.

11. The method of making a composite steel tubing according to claim 6, wherein one of the tubing sections provided has its mating surface scored prior to telescoping the tubing sections.

12. The method of making a composite steel tubing according to claim 6, wherein the outer diameter surface of the inner tubing section is scored prior to telescoping the tubing sections.

13. The method of making a composite steel tubing according to claim 6, wherein the inner diameter surface of the outer tubing section is scored prior to telescoping the tubing sections.

14. The method of making a composite steel tubing comprising the steps of:

- a. Providing two sections of welded steel tubing of substantially equivalent wall thickness, one of which sections has an outer diameter less than the inner diameter of the other;
- b. telescoping said tubing sections and locking them together at one end;
- c. changing the diameter of one of said tubing sections so as to produce a mechanical bond therebetween; and
- d. cold drawing the united tubing sections through a sizing die and over a mandrel.

\* \* \* \* \*

45

50

55

60

65